

## UNITED STATES PATENT OFFICE

OTTO KAMPS, OF AACHEN, GERMANY

## ALUMINIUM ALLOY

No Drawing. Application filed December 5, 1929, Serial No. 411,973, and in Germany October 5, 1927.

This invention relates to a process of refining an aluminium alloy which as compared with the known alloys of this kind possesses particularly valuable properties.

5 The alloy has an admixture of a cerium-copper alloy besides an admixture of thorium and nickel.

The process for refining the alloy consists in that the alloy is annealed at 535° to 480° 10 C. and subsequently submitted to a heating treatment between 300° and 50° C. in a barium-chloride bath, which is a solution of a barium-chloride salt.

These variations in temperature depend 15 less upon the actual composition of the alloy than upon the strength and expansion. Different tempering heats are selected, as strength, expansion and tempering heaters are dependent upon one another and as it is 20 possible by suitably selecting the temperatures, to give the alloy a strength and expansion of a certain value determined by the use of the alloy for the actual constructional purpose. In the case of an alloy with a nickel 25 content of 1% and a thorium content of 0.2% a temperature of 180° C. should be chosen. The contents of the alloy within the limits indicated are necessary in the case of use of the 30 alloy resisting sea water and atmospheric influences. The nickel and thorium contents are absolutely indispensable therefor.

The new alloy is an extremely thin liquid in molten state and surpasses the known aluminium alloys in regard to its possibilities of use as it can be cast to paper thickness in sand and enables in the most complicated castings an absolutely perfect shape without blow holes or shrinking holes. The strength of the castings made from this alloy 40 varies according to the thickness of the walls between 16 and 22 kgs. per square millimetre. By treating the alloy according to the refining process indicated the strength of the material is increased. Besides its homogeneous, 45 fine crystalline grain the alloy is remarkable

for its extremely high resisting properties against acids, saline solutions and sea water. These properties permit of an extensive working of the alloy in cast and rolled form.

The material produced from the alloy practically does not oxidize, is clean and does not mark. It can be easily rolled and in rolled condition attains a strength of 40 to 45 kgs. per square millimetre with expansions of 11 to 15%. By subsequent compression by rolling 55 and the like the strength of the alloy may be increased to 50 to 55 kgs. per square millimetre. Plates may be rolled from the alloy in any length and width without edge cracking and without soiling the rolls. Of particular importance is the fact that the scrap may be repeatedly melted down and the quality of the material is considerably improved thereby in that it becomes more and more homogeneous. The alloy may be used with great success for splash and chill castings as the thin liquidity allows the most complicated castings to be made without trouble with an accuracy of 1/100 mm. If 1.5% nickel be added to the new alloy the shrinkage is reduced to such an extent that the alloy is suitable as material for internal pistons of combustion engines. With suitable percentages of nickel and thorium the alloy has given excellent results. The admixture of thorium increases 70 the critical recrystallization temperature, so that hot stressed rolled materials may be subjected in work to higher temperatures without any danger of hot brittleness by reducing the strength properties. 75

The alloy preferably has the following composition:—

0.3 to 1.5% nickel, 0.05 to 0.9% thorium, 85 6.8% binary copper-cerium alloy containing 90% copper and 10% cerium, 0.4 to 0.8% manganese and the remainder aluminium with the usual commercial iron content tolerances.

I claim:—

A heat treated aluminium alloy consisting 90 of an alloy containing 5% copper, 0.3% nick-

el, 0.1% thorium, 6.8% binary copper-cerium alloy containing 90% copper and 10% cerium, having a fine crystalline structure and the remainder aluminium quenched from a temperature of from 535 to 480° C. to room temperature in a barium chloride bath and subsequently submitted to a heating treatment between 300 and 50° C. to produce steel hardness.

10 In testimony whereof I affix my signature.  
OTTO KAMPS.